

## UNITED STATES PATENT OFFICE.

ARTHUR Z. PEDERSEN, OF WEST ORANGE, NEW JERSEY, ASSIGNOR, BY MESNE ASSIGNMENTS, TO MADSENELL CORPORATION, OF NEW YORK, N. Y., A CORPORATION OF NEW YORK.

## METHOD OF COATING WITH METALS AND RESULTING PRODUCTS.

No Drawing. Application filed May 14, 1920, Serial No. 381,435. Renewed November 10, 1923.

To all whom it may concern:

Be it known that I, ARTHUR Z. PEDERSEN, a citizen of the United States, and a resident of the town of West Orange, county 5 of Essex, State of New Jersey, have invented an Improvement in Methods of Coating with Metals and Resulting Products, of which the following is a specification.

My invention relates to improvements in 10 methods of preparing metallic surfaces for receiving adherent coatings of metal and to the products resulting from such improved methods. My invention is particularly applicable in coating iron or steel articles with 15 another metal, such as nickel, whether by electro-deposition, fusion, or otherwise.

By way of illustration, I shall describe 20 my invention as applied to the coating of iron or steel surfaces with nickel by any of the usual or well-known methods of electro-depositing nickel. It is, however, to be understood that my invention is not limited to this particular application which is herein set forth by way of example only.

25 I have discovered that by employing the surface of the metallic object to be coated as an anode in strong sulphuric acid, a new and unexpected result is obtained which renders the subsequent metallic coating remarkably adherent and gives to it certain other desirable qualities, as, freedom from blistering on heating, and the like, of considerable practical and commercial importance. I prefer to employ sulphuric acid of more than 30 about 75%, usually of more than about 85%, strength. In particular, I find that anhydrous, or substantially anhydrous, sulphuric acid is very desirable for the treatment 35 of the surface of a steel object preparatory to receiving a coating of another metal, such as nickel. During this operation there is very little gassing, very little of the metal is eaten away, and no undesirable odor is generated.

40 The above operation not only cleans the surface very thoroughly, removing grease, vegetable, animal, and mineral oils, but also brings about a condition of the surface thus treated which renders the coatings unusually 45 sound and adherent. The exact cause of this phenomenon is not clear, and I do not wish to be limited to any particular theory or explanation of the action of the strong sul-

phuric acid on the surface serving as an anode. 55

In carrying out this operation, I use a vessel analogous to that used for the electro-deposition of metals or for operating what is known in the art as an "electric cleaner" in which the object whose surface 60 is to be prepared for receiving a metallic coating is so connected as to serve as the anode, while, for the cathode, I use either another piece of steel, or preferably a sheet 65 of lead.

The electrical characteristics of such a cell are peculiar and unusual. Preferably, I employ a line voltage of less than about 42 volts, since if the line voltage equals or exceeds about 42 volts, excessive arcing takes 70 place which may injure the article being treated and may have other undesirable effects. Assuming, for example, a line voltage of about 20 volts, there is initially a flow of current amounting to about 30 amperes per 75 square foot, where either anhydrous, or substantially anhydrous sulphuric acid or 66° Baumé sulphuric acid, that is, sulphuric acid approximately 96% strong, is employed in the bath. For a few seconds the current 80 density drops slightly, then there is momentarily a sudden and slight increase in current density, after which the current density continues to continually diminish until after about ten minutes, when the operation is 85 complete, and when the current density will be found to be generally less than one ampere per square foot, or even nearly zero. This condition constituting a substantial 90 condition of equilibrium in the cell after the period of time set forth above, indicates that the voltage impressed on the cell is at least equal to the polarization voltage of the cell, in this case apparently 20 volts.

As a result of the treatment set forth, even 95 where the surface is initially coated with grease and oxide, the treated surface, after a brief shaking in water, is found to be of a clean gray metallic lustre, which receives the metallic coating readily. The coating is 100 found to be remarkably adherent and the object will be found not to readily blister or separate from its coating on heating, or in use.

It is, of course, to be understood that my 105 invention is not limited to the particular

embodiment thereof herein set forth by way of example merely.

What I claim is:

1. The method of preparing metallic surfaces to receive adherent metallic coatings which comprises making the object to be coated the anode in a bath containing sulphuric acid of more than about 75% strength.
- 10 2. The method of preparing metallic surfaces to receive adherent metallic coatings which comprises making the object to be coated the anode in a bath containing sulphuric acid of more than about 85% strength.
- 15 3. The method of preparing metallic surfaces to receive adherent metallic coatings which comprises making the object to be coated the anode in a bath containing sub-
- 20 stantially anhydrous sulphuric acid.

4. The method of preparing metallic surfaces to receive adherent metallic coatings which comprises making the object to be coated the anode in a bath containing sulphuric acid of more than about 75% <sup>25</sup> strength, and impressing on the cell thus formed a voltage at least equal to the polarization balance voltage of the cell.

5. The method of preparing metallic surfaces to receive adherent metallic coatings <sup>30</sup> which comprises making the object to be coated the anode in a bath containing substantially anhydrous sulphuric acid, and impressing on the cell thus formed a voltage at least equal to the polarization balance <sup>35</sup> voltage of the cell.

In testimony whereof, I have signed my name to this specification this eleventh day of May, 1920.

ARTHUR Z. PEDERSEN.